

# United States Patent Office

3,244,603

Patented Apr. 5, 1966

1

3,244,603

## ELECTRODEPOSITION OF A NICKEL-MANGANESE ALLOY

William B. Stephenson, Jr., Cincinnati, and Edward R. Farmer, Reading, Ohio, assignors to General Electric Company, a corporation of New York  
No Drawing. Filed June 8, 1962, Ser. No. 209,963  
6 Claims. (Cl. 204—43)

This invention relates to a nickel base, nickel-manganese alloy and, more particularly, to an electrodeposited nickel-manganese alloy suitable for use in a method of electroforming articles.

Electroforming, which is sometimes referred to as electrofabricating, is a process which has been used to create articles of a variety of sizes and shapes. Examples of such articles are hypodermic needles, microscopic grooves of high fidelity record stampers, huge dish like molds for forming plastic canopies, fountain pen caps and electrolyte. When accurately controlled, the electroforming process allows for the formation of intricate parts with accurate dimensions and at relatively low cost. However, one of the problems which must be solved before such a process can be adapted to the manufacture of articles to operate under highly stressed conditions such as in jet engines, is that the metal or metal alloy which is electrodeposited to form the desired article must have sufficient strength and ductility to withstand the difficult conditions to which an article would be subjected in operation.

The present invention, in one form, has recognized that a particular aqueous electroplating bath can be used to develop a nickel base, nickel-manganese alloy of unusual strength characteristics.

Electroplating, of course, is a very old art and the plating of nickel and manganese in the same bath was reported in U.S. Patent 1,026,628—Leuchter in 1912. U.S. Patent 2,377,321—Brown et al., and U.S. Patent 2,905,601, mention the formation of a nickel-manganese alloy in the electrodeposition art.

Although an electrodeposited alloy of nickel and manganese has been produced there still exist a number of difficulties in producing such an electrodeposit in a crack-free condition and sufficiently thick when formed as a structural member. However, it has been recognized that the co-electrodeposition of nickel and manganese under certain conditions can result in an unusual crack-free material which can have strength and ductility.

It is a principal object of this invention to provide an electrodeposited nickel-manganese alloy having unusual strength and ductility characteristics.

Another object is to provide an electrolyte and a method for electrodepositing a nickel-manganese alloy into an article shape which has strength characteristics unusual for an electroformed article.

These and other objects and advantages will become more apparent from the following more detailed discussion and examples which are exemplary of rather than limitations on the scope of the present invention.

Briefly, the present invention provides an electroformed Mi-Mn alloy including less than 1 weight percent manganese and preferably consisting essentially of 0.03—0.8 weight percent manganese with the balance nickel. Strong articles of the alloy of this invention can be electroformed from an aqueous sulfamate nickel electroplating bath in which the manganese metal content is about 2—5 ounces per gallon and the nickel metal content is about 10—12 ounces per gallon, with the bath being operated at a temperature above about 120° F. preferably at a current density of between about 20—75 amps per square foot.

Although a variety of nickel electroplating baths or electrolytes are well known in the art of electroplating,

2

it was recognized that sulfamate type baths produce electrodeposits better suited for high temperature applications. This was demonstrated by testing a number of different nickel plating solutions two of which are represented as follows:

### Aqueous solution A

|                 |              |           |
|-----------------|--------------|-----------|
| Nickel metal    | oz./gal.     | 10.0—10.5 |
| Boric acid      | do           | 4.5—5.0   |
| pH              |              | 4.0—4.2   |
| Temperature     | ° F.         | 140       |
| Current density | amps/sq. ft. | 50        |

<sup>1</sup> As nickel sulfamate.

### Aqueous solution B

|                   |              |     |
|-------------------|--------------|-----|
| Nickel sulphate   | oz./gal.     | 24  |
| Ammonium chloride | do           | 3.5 |
| Boric acid        | do           | 4.0 |
| pH                |              | 3.5 |
| Temperature       | ° F.         | 130 |
| Current density   | amps/sq. ft. | 50  |

The following Table I presents average ultimate tensile strength (UTS) data in thousands of pounds per square inch at three different temperatures with the electrodeposited material of about 0.030" thick having been pre-treated under several different conditions.

TABLE I

| 30 | Solution | Temp.<br>(° F.) | Anneal<br>Temp.<br>(° F.) | Avg.<br>UTS<br>(k.p.s.i.) | Elongation<br>(percent) |
|----|----------|-----------------|---------------------------|---------------------------|-------------------------|
| 35 | A        | Room            | As plated                 | 141                       | 11                      |
|    | B        | Room            | As plated                 | 112                       | 5                       |
|    | A        | 750             | 750                       | 117                       | 15                      |
|    | B        | 750             | 750                       | 75                        | 25                      |
|    | A        | 750             | 750                       | 69                        | 12                      |
|    | B        | 750             | 750                       | 36                        | 11                      |
|    | A        | 750             | 1,100                     | 39                        | 31                      |
|    | B        | 750             | 1,100                     | 33                        | 5                       |
|    | A        | 1,100           | 1,100                     | 18                        | 6                       |
| 40 | B        | 1,100           | 1,100                     | 7                         | 18                      |

It is readily recognized that up to a temperature of about 1100° F., the sulfamate type of bath represented by Aqueous Solution A has better characteristics for high temperature operation.

It was recognized from the following Aqueous Solution C that the addition of manganese as an alloying element with nickel resulted in unusual properties.

The electrolyte solution used was as follows:

### Aqueous solution C

| 55                             |  | Oz./gal. |
|--------------------------------|--|----------|
| Nickel metal (as sulfamate)    |  | 10.5     |
| Manganese metal (as sulfamate) |  | 4.0      |
| Boric acid                     |  | 4.0      |

Aqueous Solution C at a pH of 3.5 and a temperature of 140° F. was used at a current density of about 50 amps/sq. ft. with depolarized nickel anodes to produce a nickel-manganese alloy sheet 8" x 10" x 0.030". This material of 0.4 weight percent Mn, balance Ni showed that the hardness and heat stability of nickel alone is changed markedly by the inclusion of manganese.

As a result of this initial discovery, a number of sample solutions were tested. Some of these are presented in Table II along with the conditions under which sheets of 0.030 inch thick alloy was produced. Table III gives the weight percent of manganese in each sheet, the balance of which was nickel. Comments as well as hardness figures regarding the physical condition of the electrodeposited alloy are included.

TABLE II.—ELECTROLYTE BATH

| Example | Ni<br>(oz./gal.) | Mn<br>(oz./gal.) | pH  | Temp.<br>(° F.) | Current<br>density<br>(amps./ft. <sup>2</sup> ) |
|---------|------------------|------------------|-----|-----------------|-------------------------------------------------|
| 1       | 11.7             | 8.5              | 3.5 | 130             | 35                                              |
| 2       | 11.7             | 6.2              | 3.5 | 130             | 35                                              |
| 3       | 11.5             | 5.2              | 3.5 | 130             | 35                                              |
| 4       | 11.7             | 3.9              | 3.5 | 130             | 35                                              |
| 5       | 11.8             | 3.2              | 3.5 | 130             | 35                                              |
| 6       | 11.7             | 2.3              | 3.5 | 130             | 35                                              |
| 7       | 11.7             | 3.9              | 3.5 | 130             | 20                                              |
| 8       | 11.7             | 3.9              | 3.5 | 130             | 50                                              |
| 9       | 12.0             | 4.0              | 3.5 | 90              | 35                                              |
| 10      | 11.7             | 3.9              | 3.5 | 120             | 35                                              |
| 11      | 11.7             | 3.9              | 3.5 | 140             | 35                                              |
| 12      | 11.7             | 3.9              | 3.5 | 150             | 35                                              |
| 13      | 11.7             | 3.9              | 3.5 | 160             | 35                                              |
| 14      | 12.0             | 4.0              | 5   | 130             | 35                                              |
| 15      | 11.7             | 3.9              | 3   | 130             | 35                                              |
| 16      | 12.0             | 4.0              | 2   | 130             | 35                                              |
| 17      | 12.0             | 4.0              | 1   | 130             | 35                                              |
| 18      | 11.7             | 3.9              | 3.5 | 140             | 50                                              |
| 19      | 12.0             | 4.0              | 3.5 | 140             | 75                                              |

TABLE III.—PLATED DEPOSIT

| Example | Mn (Wt. percent) | Stress <sup>1</sup> | Hardness, R <sub>c</sub> | Physical condition <sup>2</sup> |
|---------|------------------|---------------------|--------------------------|---------------------------------|
| 1       | 1.2              | H                   | 51                       | D.                              |
| 2       | 1.2              | H                   | 47                       | D.                              |
| 3       | 0.8              | M                   | 43                       | C.                              |
| 4       | 0.6              | S                   | 36                       | A.                              |
| 5       | 0.5              | S                   | 34                       | A.                              |
| 6       | 0.3              | VS                  | 20                       | A.                              |
| 7       | 0.1              | VS                  | 26                       | A.                              |
| 8       | 0.7              | M                   | 37                       | A.                              |
| 9       | 4.5              | H                   | 43                       | D.                              |
| 10      | 0.9              | H                   | 43                       | D.                              |
| 11      | 0.6              | S                   | 34                       | A.                              |
| 12      | 0.2              | S                   | 31                       | A.                              |
| 13      | 0.03             | S                   | 29                       | A.                              |
| 14      | 0.6              | M                   | 41                       | B.                              |
| 15      | 0.4              | S                   | 34                       | A.                              |
| 16      | 0.5              | S                   | 37                       | A.                              |
| 17      |                  | VS                  |                          | E.                              |
| 18      | 0.4              | S                   | 36                       | A.                              |
| 19      | 0.4              | S                   | 38                       | A.                              |

<sup>1</sup> H=high. M=moderate. S=slight. VS=very slight.

<sup>2</sup> A=Sound. B=Slightly brittle. C=fine cracks along edges. D=cracked and brittle. E=many gas pits, soft and granular.

It is to be noted that with less than 1 weight percent manganese, the hardness and heat stability of the nickel-manganese alloy is markedly changed. Generally, the manganese content decreases as the temperature of the electroplating bath increases while the manganese content increases with current density. However, the manganese content was generally unaffected by variations in pH between about 1 and 5, although the physical condition of the alloy deposited at a pH of 1 was unusually poor as compared with that produced at a pH of 2. Examples 1-6 represent variations in the manganese content of the bath; Examples 7, 8, 18 and 19 represent variations in the current density at two different temperatures; Examples 9-13 represent variations in bath temperature and Examples 14-17 represent the effect of change in pH.

The hardness data shows that an alloy hardness of above about 40 Rockwell C (R<sub>c</sub>) results in too high a stress level in the alloy and leads to cracks in the material. Furthermore, a manganese content below about 0.8 weight percent of the alloy results in a sound, strong alloy whereas alloys containing manganese at or above about 1.2 weight percent are brittle and highly stressed.

From aqueous solution C and those in Table II, it has been found that the manganese metal content in the electrolyte of this invention lies in the range of about 2-5 ounces per gallon and the nickel metal content lies in the range of about 10-12 ounces per gallon. Both of

the metals are present in the aqueous bath as metal sulfamate along with an agent such as boric acid normally used in nickel electroplating solutions. Furthermore, the temperature should be maintained above 120° F., generally within the range of 120-160° F. and preferably in the range of 130-150° F. The pH between 2-5 resulted in satisfactory alloy with extraordinary material being produced at a pH between about 2-4. Excellent material was deposited at current densities between 20-75 amps per square foot but the electrodeposition of the nickel-manganese alloys from an aqueous bath at a temperature of 120° F. or less resulted in a highly stressed material which was cracked and brittle.

The data shows that an electroformed Ni-Mn alloy deposited from a sulfamate solution and including less than 1 weight percent Mn and preferably consisting essentially of 0.03-0.8 weight percent manganese with the balance nickel has unusual characteristics which were unrecognized prior to the present invention.

In order to evaluate the strength properties of the alloy of the present invention, a series of 8" x 10" rectangles 0.030" thick were prepared from the following sulfamate plating bath and under the listed conditions to result in a composition of 0.5 weight percent manganese with the balance nickel.

Nickel metal content (as sulfamate) oz./gal. 10.5-11.0  
Manganese metal content (as sulfamate) oz./gal. 3.5-4.0  
pH 3.5-4  
Temperature ° F. 135-140  
Current density amps/sq. ft. 50  
Hardness R<sub>c</sub> 35.40

Prior to testing, the alloy rectangles were stabilized by heating at 800° F. for 16 hours and then air cooling to insure that no changes in the material would take place as a result of exposure to the test temperatures and to remove any entrapped hydrogen which is known to exist in slight amounts in the as-plated condition.

It has been found that any brittleness which might exist in the as-plated condition within the range of the alloy of this invention, is caused mainly by cathodic hydrogen content. In such a case, adequate ductility can be imparted to such alloy by a low temperature anneal to degas the material without loss in strength.

The specimens made from the alloy rectangles were 0.350" wide by 2" gage length. The following Table IV gives the average tensile properties of such specimens.

TABLE IV.—TENSILE PROPERTIES

| Temp. (° F.) | Avg. UTS (k.p.s.i.) | Avg. elongation (percent) | Avg. hardness (R <sub>c</sub> ) |
|--------------|---------------------|---------------------------|---------------------------------|
| Room         | 179                 | 5.4                       | 39                              |
| 200          | 165                 | 4.0                       | 37                              |
| 400          | 130                 | 5.6                       | 36                              |
| 600          | 99                  | 18.0                      | 37                              |

It is to be noted that the Ni-Mn alloy of the present invention is substantially stronger than the Ni-metal specimens, the data for which is shown in Table I.

A photomicrograph of a cross section of the electro-deposited Ni-Mn alloy of this invention have shown that the alloy does not have the conventional crystal structure that would normally be attributed to this type of alloy. The appearance of the structure is similar to that of untempered martensite. It is believed that the fine as-plated grain size is primarily responsible for the high mechanical properties of this alloy.

Although this invention has been described in connection with specific examples, it will be readily recognized by those skilled in the art of electrodeposition, the variations and modifications possible within the scope of the invention described.

What is claimed is:

1. An alloy of nickel and manganese electrodeposited from a sulfamate electrolyte and consisting essentially of 0.03-0.8 weight percent manganese with the balance nickel, the alloy having a hardness of less than about 40 Rockwell C. 5
2. An alloy of nickel and manganese electrodeposited from a sulfamate electrolyte and consisting essentially of 0.03-0.8 weight percent manganese, with the balance nickel, the alloy having a hardness between 20-40 Rockwell C. 10
3. For electrodepositing an Ni-Mn alloy of up to about 1 weight percent manganese, an aqueous electrolyte consisting essentially of:
  - a manganese metal content of 2-5 oz./gal., and 15
  - a nickel metal content of 10-12 oz./gal.;
  - the manganese metal and the nickel metal being in the electrolyte in the form of sulfamates; and
  - the electrolyte having a pH of about 2-5.
4. For electrodepositing an Ni-Mn alloy of up to about 1 weight percent manganese, an aqueous electrolyte consisting essentially of:
  - a manganese metal content of 3.5-4 oz./gal.; and 20
  - a nickel metal content of 10.5-11 oz./gal.;
  - the manganese metal and the nickel metal being in the electrolyte in the form of sulfamates; and
  - the electrolyte having a pH of about 3.5-4.
5. In a method for electrodepositing an Ni-Mn alloy, the steps of:
  - electrolyzing an aqueous electrolyte consisting essentially of a manganese metal content of about 2-5 oz./gal. and a nickel metal content of about 10-12 oz./gal., the manganese metal and the nickel metal being in the electrolyte in the form of sulfamates; and 30
  - during electrolyzing, maintaining the electrolyte pH at about 2-5 and the temperature above about 120° F. 35

6. In a method for electrodepositing an Ni-Mn alloy, the steps of:
  - electrolyzing at a current density of about 20-75 amps/sq. ft. an aqueous electrolyte consisting essentially of a manganese metal content of 2-5 oz./gal. and a nickel metal content of 10-12 oz./gal., the manganese metal and the nickel metal being in the electrolyte in the form of sulfamates; and
  - during electrolyzing, maintaining the electrolyte pH at 2-5 and the temperature between 120 and 160° F.

#### References Cited by the Examiner

##### UNITED STATES PATENTS

|           |         |               |       |        |
|-----------|---------|---------------|-------|--------|
| 1,026,628 | 5/1912  | Leuchter      | ----- | 204-43 |
| 2,318,592 | 5/1943  | Cupery        | ----- | 204-52 |
| 2,377,321 | 6/1945  | Brown et al.  | ----- | 204-43 |
| 2,458,839 | 1/1949  | Dyer          | ----- | 204-43 |
| 2,489,523 | 11/1949 | Clifton       | ----- | 204-43 |
| 2,798,038 | 7/1957  | Dean          | ----- | 204-45 |
| 2,805,192 | 9/1957  | Brenner       | ----- | 204-43 |
| 2,905,601 | 9/1959  | Rinker et al. | ----- | 204-43 |
| 2,927,066 | 3/1960  | Schaer        | ----- | 204-43 |
| 3,027,309 | 3/1962  | Stephen       | ----- | 204-43 |

#### OTHER REFERENCES

Metal Finishing Guidebook Directory, 29th edition, page 344, 1961.

Piontelli et al., Proc. of the Third Int'l. Conference on Electrodeposition, Electrodepositors Technical Society, September 1947, pp. 121-125.

JOHN H. MACK, *Primary Examiner.*

JOHN R. SPECK, *Examiner.*

G. KAPLAN, *Assistant Examiner.*